

## UNITED STATES PATENT OFFICE

2,092,451

## ELECTROLYTIC PRODUCTION OF LEAD

Allan Robert Gibson, Redland, Bristol, and Stanley Robson, Shirehampton, Bristol, England, assignors to The National Smelting Company Limited, London, England, a limited-liability company of England

No Drawing. Application October 12, 1935, Serial No. 44,804. In Great Britain November 5, 1934

## 3 Claims. (Cl. 204—19)

This invention relates to the treatment of metalliferous materials containing lead and sulphur.

It has been proposed hitherto to add a sulphide ore such as lead sulphide to a fused lead chloride bath and by electrolysis to recover the metal and elementary sulphur from the respective electrodes. We have found that in order to obtain a constant production of elementary lead and sulphur with the least consumption of electrical energy, a comparatively low concentration of lead sulphide is generally necessary, but the concentration is dependent upon the temperature of the melt and the current density applied.

According to the present invention lead and sulphur are separated from metalliferous materials containing them (for example, galena) by submitting to electrolysis fused lead chloride containing the said metalliferous material, the process being characterized in that the concentration of lead sulphide in the melt is maintained between 1% and 10% and the current density is so adjusted for this range of concentrations that as the concentration is increased above 1%, the current density is varied between 500 and 1000 amps. per square foot. Under these conditions the temperature of the electrolyte is maintained between 500 and 600° C.

By this means the formation of sulphur chloride is avoided on the one hand and the current efficiency is maintained on the other, so that the ohmic resistance of the melt is sufficient to enable an impressed voltage above the decomposition voltage necessary to operate the process, to be applied.

We have found that satisfactory conditions are obtained with a lead sulphide concentration in the melt of 3% at a temperature of 550° C. and employing a current density of 600 to 750 amps. per square foot. If the process is conducted at the lower end of the ranges given above, i. e. with a current density of 500 amps. per square foot a temperature of 500 to 600° C. and a galena concentration of 1 to 2%, electrolysis proceeds normally. If, however, with the current density and temperature remaining constant, the galena concentration be progressively increased the ohmic resistance of the melt is decreased until a point is reached in the neighbourhood of 3% galena concentration at which normal electrolysis is suspended and the sulphur is retained by the melt presumably in the form of di- or poly-sulphide of lead. Beyond this point if the galena concentration is increased the current density must be correspondingly increased until with a

concentration of 5% the current density should be about 750 amps. per square foot. With this increase of current density the temperature of the melt will naturally rise. However, normal electrolysis of the cell may be restored by cessation of the feed of lead sulphide. Sulphur will then be liberated at the anode, and PbS reformed at the cathode by electrolytic decomposition of the complex, until eventually only lead sulphide (PbS) remains in the melt, when normal electrolysis with the formation of the lead at the cathode and sulphur vapour at the anode is resumed.

In one way of carrying out the process of the invention lead chloride is melted and maintained in the fused condition in any well known type of cell suitable for the electrolysis of fused salts, and galena is added from time to time to maintain a concentration of about 3-5%. The current density employed for this concentration is about 750 to 1000 amps. per square foot of electrodes surface. We prefer to employ a column of bi-polar electrodes with a gap of  $\frac{1}{2}$  inch. The voltage drop over each gap is 1.2 to 1.4. The supply of galena to the cell is regulated according to the voltage over the cell, the temperature being constant. At a fixed temperature the voltage over the cell serves as a guide to the concentration of galena in the melt and this may be maintained approximately constant by additions of galena during operation. If in this way too much galena is added it will also be readily observed by the decrease or cessation of sulphur at the anode owing to the formation of complex sulphides in the melt, a condition which may be remedied by cessation of the feed or increase of the current density. It is desirable to employ mechanical agitation to keep the composition of the electrolyte constant, because the agitation due to thermal convection currents only is insufficient for this purpose. Under these conditions lead is recovered with a consumption of 750 to 800 kilowatt hours per ton of lead, and the sulphur is recovered in the elementary state.

According to a feature of the invention the mixture may be subjected to a preliminary electrolysis to remove metals electro-negative to lead, in particular silver.

We have found it desirable to make the additions of galena to an inner compartment which can be sealed from the electrolysis proper. In this inner compartment the gangue formed on the addition of galena may be readily skimmed from the melt. The preliminary electrolysis may also be carried out in the inner compartment while it is sealed from electrolysis proper, or

purification may be effected by allowing the mixture to pass through a molten lead seal between the inner compartment and the cell proper.

Using bi-polar electrodes the passage of the current causes separation of molten lead at the cathode surfaces and gaseous sulphur at, or near, the anode. The sulphur is collected by means of a suitable reflux condenser, and the lead is removed in the molten state from the cell by means of a suitably designed siphon.

The gangue removed from the melt will contain some lead chloride, and this may be removed by volatilization of lead chloride and the fume condensed on galena and returned to the cell.

What we claim is:—

1. A process for separating lead and sulphur from metalliferous materials containing lead sulphide which comprises submitting to electrolysis fused lead chloride containing the said metalliferous material with a concentration of lead sulphide in the melt between 1% and 10% and at a current density between 500 and 1000 amps. per square foot, the current density varying proportionately to the lead sulphide concentration.

2. A process for separating lead and sulphur from metalliferous materials containing lead sulphide comprising submitting a solution of 3 to 5% of lead sulphide in lead chloride to electrolysis at a current density between 750 and 1000 amps. per square foot so as to cause sulphur vapour to be given off at the anode, adding further lead sulphide-containing material to the melt and regulating the rate of addition and the current density so that the flow of sulphur vapour from the neighbourhood of the anode remains substantially constant. 5 10

3. A process for separating lead and sulphur from metalliferous materials containing lead sulphide which comprises electrolyzing in a cell employing bi-polar electrodes with a voltage drop of 1.2 to 1.4 over each gap, a solution of 3% to 5% of lead sulphide in lead chloride, adjusting the current density between 750 and 1000 amps. per square foot according to the concentration 15 20 of lead sulphide so that a substantially constant flow of sulphur vapour is maintained from the neighbourhood of the anode.

ALLAN ROBERT GIBSON. 25  
STANLEY ROBSON.